# EUROPEAN PATENT SPECIFICATION

(11) **EP 4 067 530 B1**
(45) Date of publication and mention of the grant of the patent: **13.08.2025**
(21) Application number: 20893836.5
(22) Date of filing: 28.09.2020
(51) Int. Cl.: C23C 2/12, C22C 38/18, C23C 2/26, C23C 2/40, B21D 22/02, B21D 22/20, C21D 8/02, C21D 1/18, C22C 38/02, C22C 38/04, C22C 38/06, C22C 38/24, C22C 38/26, C22C 38/28, C22C 38/32, C21D 1/673, C21D 1/74, C21D 7/13, C21D 9/46, C22C 38/38

(54) **THERMOFORMED COMPONENT HAVING EXCELLENT COATING ADHESION, AND MANUFACTURING METHOD THEREFOR**
THERMOGEFORMTE KOMPONENTE MIT AUSGEZEICHNETER BESCHICHTUNGSHAFTUNG UND VERFAHREN ZU IHRER HERSTELLUNG
COMPOSANT THERMOFORMÉ AYANT UNE EXCELLENTE ADHÉRENCE DE REVÊTEMENT ET SON PROCÉDÉ DE FABRICATION

(30) Priority: 29.11.2019 CN 201911202456
(43) Date of publication of application: 05.10.2022
(73) Proprietor: BAOSHAN IRON & STEEL CO., LTD., Shanghai 201900 (CN)
(72) Inventor: TAN, Ning, Shanghai 201900 (CN); LIU, Hao, Shanghai 201900 (CN); HONG, Jiyao, Shanghai 201900 (CN); JIN, Xinyan, Shanghai 201900 (CN)
(74) Representative: Kuhnen & Wacker Patent- und Rechtsanwaltsbüro PartG mbB
(86) International application number: PCT/CN2020/118368
(87) International publication number: WO 2021/103805

(56) References cited:
- EP-A1- 3 070 187
- EP-A1- 3 354 360
- CN-A- 105 829 578
- CN-A- 106 165 112
- CN-A- 106 466 697
- CN-A- 110 117 167
- KR-A- 20130 110 532

## Description

### TECHNICAL FIELD

The present invention relates to a material and a manufacturing method therefor, and particularly relates to a thermoformed material and a manufacturing method therefor.

### BACKGROUND ART

In recent years, the application of thermoformed component in automobile industry has become very important. Especially, with respect to safety structural parts of automobile, it has irreplaceable advantages in some parts with high strength and complex shape. The materials used for thermoformed components are divided into those with coating and those without coating. The main purpose of the coating is to prevent the oxidation of the steel plate surface during the hot stamping process. The formed components can be directly coated and welded for use. At present, the materials without coating must be subject to surface shot peening after thermoforming to remove the oxide layer generated on the surface, otherwise it will affect the subsequent coating and welding of parts. The surface of materials hot-dipped with aluminum coating cannot be phosphated normally after thermoforming. The adhesion of paint film after electrophoresis depends entirely on the surface morphology of the coating. During the use of existing materials, there will be the problem that the coating adhesion cannot meet the use.

For example, the Chinese patent document with the publication number of CN 104 651 590 A and the publication date of May 27, 2015, entitled "process for manufacturing stamped products, and stamped products prepared from the same" discloses a thermoforming material coated with aluminum or aluminum alloy and its manufacturing method. The method specifically controls the thickness and five-layer structure of the coating to ensure the welding performance of thermoformed component.

For another example, the Chinese patent document with the publication number of CN 108 588 612 A and the publication date of September 28, 2018, entitled "hot-stamping forming component, pre-coating steel-plating plate for hot-stamping forming, and hot-stamping forming process" discloses a hot-stamping formed component. In the technical solution disclosed in the patent document, the thickness of the coating is reduced and the protective effect of the coating is also reduced. Therefore, the fluctuation of the thermoforming process is easy to affect the surface performance of the component, thus affecting the subsequent service performance.

For another example, the Chinese patent document with the publication number of CN 101 583 486 A and the publication date of November 18, 2009, entitled "coated steel strip, methods of making the same, methods of using the same, stamping blanks prepared from the same, stamped products prepared from the same, and articles comprising such stamped products" discloses a hot stamped product of coated steel strip and a method. The technical solution disclosed in the patent document includes heating, transferring and cooling, but does not involve the hot stamping process, which will lead to the unstable quality of stamped products, such as shrinkage and cracking. The furnace atmosphere during the heating process is not controlled, which leads to the change of furnace atmosphere during the heating, especially the large change of oxygen content, which makes the appearance color of products easy to change. In the actual production, it is found that the appearance color of stamped products obtained from the same incoming materials under the same process is quite different. Moreover, the published patent applications EP 3 070 187 A1, EP 3 354 360 A1 and CN 106 466 697 A disclose steel sheets according to prior art.

### SUMMARY OF INVENTION

An object of the present invention is to provide a thermoformed component having excellent coating adhesion. The thermoformed component has good paintability, good coating adhesion and good corrosion resistance, and is very suitable for automotive parts, such as front and rear doors, left and right anti-collision rods/beams, front and rear bumpers, A-pillar reinforcing plates, B-pillar reinforcing plates, floor middle channels, etc.

To achieve the above object, the present invention provides a thermoformed component having excellent coating adhesion, comprising a substrate layer and an aluminum coating coated on at least one surface of the substrate layer, wherein the average roughness Ra of a surface of the thermoformed component is between 1.0 µm and 3.0 µm, the peak-to-valley height Rt is between 8 µm and 30 µm, and the roughness peak count Rpc is greater than or equal to 50, wherein the mass percentage of chemical elements of the aluminum coating is: Si: 4~14%, Fe: 0~4%, Mg: 0~10%, Zn: 0~20%, and a balance of Al and other unavoidable impurities, wherein the aluminum coating comprises a diffusion layer adjacent to the substrate layer and an alloy layer on the surface of the aluminum coating, wherein the ratio of the thickness of the diffusion layer to the total thickness of the aluminum coating is 0.08-0.5; wherein the mass percentage of chemical elements of the substrate layer is: C: 0.01 -0.8%, Si: 0.05~1.0%, Mn: 0.1 ~5%, P≤0.3%, S≤0.1%, Al<0.3%, Ti≤0.5%, B: 0.0005~0.1%, Cr: 0.01 ~3%, Nb≤0.5%, V≤0.5%, and a balance of Fe and other unavoidable impurities.

In the technical solution of the present invention, the aluminum coating comprises aluminum phase and aluminum silicon phase. In the heating process, the aluminum in the aluminum coating diffuses to the substrate layer, and the iron in the substrate layer diffuses to the aluminum coating to form Al₈Fe₂Si phase. The formation of new phase leads to a significant increase in surface roughness. With the further diffusion of iron and aluminum, Fe₂Al₅ phase is formed, and the surface roughness is basically maintained. Finally, FeAl alloy is completely formed in the aluminum coating, while the surface roughness decreases slightly.

The surface of thermoformed components after heat treatment mainly consists of Fe₂Al₅ and FeAl alloy. At the same time, because the silicon oxide, aluminum oxide and iron oxide produced by surface oxidation cannot react with phosphating solution, that is, normal phosphating coating cannot be formed, the coating adhesion of thermoformed components is completely guaranteed by the uneven structure of the surface, that is, the roughness of thermoformed components has an important impact on the coating adhesion.

The greater the surface roughness of the aluminum coating, the greater the roughness peak count Rpc value, the different diffusion paths of iron and aluminum, and the different speed of the formation of new phase, resulting in the greater the surface roughness of the formed components after heat treatment and the better the coating adhesion.

Further, in the thermoformed component having excellent coating adhesion according to one embodiment of the present invention, the thickness of the diffusion layer is ≤ 16 µm; the total thickness of the aluminum coating is ≤ 60 µm.

Further, in the thermoformed component having excellent coating adhesion according to one embodiment of the present invention, the thickness of the diffusion layer is 5~16 µm; the total thickness of the aluminum coating is 20~60 µm.

Further, in the thermoformed component having excellent coating adhesion according to one embodiment of the present invention, the average roughness Ra of the surface of the thermoformed component is 1.5~2.5 µm.

Further, in the thermoformed component having excellent coating adhesion according to one embodiment of the present invention, the peak-to-valley height Rt of the surface of the thermoformed component is 10~25 µm.

Further, in the thermoformed component having excellent coating adhesion according to one embodiment of the present invention, the roughness peak count Rpc of the surface of the thermoformed component is 50~250, such as 80~180.

Further, the surface of the thermoformed component having excellent coating adhesion of an embodiment the present invention comprises Fe₂Al₅ and FeAl alloy. Further, the surface of the thermoformed component having excellent coating adhesion of an embodiment of the present invention also comprises silicon oxide, aluminum oxide and iron oxide. Further, the surface of the thermoformed component having excellent coating adhesion of the present invention mainly consists of Fe₂Al₅ and FeAl alloy, and also comprises silicon oxide, aluminum oxide and iron oxide. Also, the content of Fe₂Al₅ in the surface of the thermoformed component having excellent coating adhesion of the present invention is higher than 40wt%.

Further, in the surface of the thermoformed component having excellent coating adhesion according to the present invention, the mass percentage of chemical elements of the aluminum coating is: Si: 4~14%, Fe: 2~4%, Mg: 0~10%, Zn: 0~20%, and a balance of Al and other unavoidable impurities.

Further, in the thermoformed component having excellent coating adhesion according to one embodiment of the present invention, the average weight of the aluminum coating is 20~120 g/m² per single surface.

Further, in the thermoformed component having excellent coating adhesion according to one embodiment of the present invention, the average weight of the aluminum coating is 30~100 g/m² per single surface.

Further, in the thermoformed component having excellent coating adhesion according to one embodiment of the present invention, the mass percentage of chemical elements of the substrate layer further meets at least one of the following:
C: 0.05~0.6%,
Si: 0.07~0.8%,
Mn: 0.3~4%,
P≤0.2%,
S≤0.08%,
Al≤0.2%,
Ti≤0.4%,
B: 0.0005~0.08%,
Cr: 0.01 ~2%,
Nb≤0.3%,
V≤0.3%.

Further, in the thermoformed component having excellent coating adhesion according to one embodiment of the present invention, the mass percentage of chemical elements of the substrate layer further meets at least one of the following:
C: 0.15~0.5%,
Si: 0.1-0.5%,
Mn: 0.5~3%,
P≤0.1%,
S≤0.05%,
Al≤0.1%,
Ti≤0.2%,
Cr: 0.01 ~1%.

Further, in the substrate layer of the thermoformed component having excellent coating adhesion according to one embodiment of the present invention, the content of Al is 0.03-0.09%, and the content of Ti is 0.01-0.2%, preferably 0.01-0.1%.

Further, in the substrate layer of the thermoformed component having excellent coating adhesion according to one embodiment of the present invention, the content of Cr is 0.1-0.8%.

Further, in the substrate layer of the thermoformed component having excellent coating adhesion according to one embodiment of the present invention, when Nb is comprised, the content of Nb is 0.001-0.1%, when V is comprised, the content of V is 0.001-0.01%.

Further, in the thermoformed component having excellent coating adhesion according to one embodiment of the present invention, the mass percentage of chemical elements of the substrate layer is: C: 0.02~0.8%, Si: 0.05~0.5%, Mn: 0.1~3%, P≤0.1%, S≤0.05%, Al: 0.04-0.09%, Ti: 0.02-0.2%, B: 0.0005~0.09%, Cr: 0.15~0.8%, Nb: 0% or 0.001-0.1%, V: 0% or 0.002-0.008%, and a balance of Fe and other unavoidable impurities.

Further, in the thermoformed component having excellent coating adhesion according to one embodiment of the present invention, the yield strength is 400~1400 MPa, the tensile strength is 500~2100 MPa, and the elongation is ≥4%.

Preferably, in the microstructure of the substrate of the thermoformed component having excellent coating adhesion of the present invention, the volume percentage of martensite is ≥70%, preferably ≥85%, more preferably ≥95%.

Accordingly, another object of the present invention is to provide a manufacturing method for the above thermoformed component having excellent coating adhesion, and through the manufacturing method, thermoformed component having excellent coating adhesion can be obtained.

To achieve the above object, the present invention provides a manufacturing method for the above thermoformed component having excellent coating adhesion, comprising the following steps:
(1) immersing a substrate in an aluminum coating solution to obtain a plate having an aluminum coating on a surface thereof, wherein the average weight of the aluminum coating is 20~120 g/m² per single surface, wherein the mass percentage of chemical elements of the substrate is: C: 0.01 -0.8%, Si: 0.05~1.0%, Mn: 0.1~5%, P≤0.3%, S≤0.1%, Al<0.3%, Ti≤0.5%, B: 0.0005~0.1%, Cr: 0.01~3%, Nb≤0.5%, V≤0.5%, and a balance of Fe and other unavoidable impurities, and wherein the mass percentage of chemical elements of the aluminum coating solution is: Si: 5~11%, Fe: 2~4%, Zn: 0~15%, Mg: 0~8%, and a balance of Al and other unavoidable impurities;
(2) leveling: using a leveling roller having a roughness Ra of 0.5~3.0 µm to level the plate, and controlling the leveling elongation ≤2.0%, so that the surface thermal radiation coefficient of the plate is 0.1~0.8, the surface roughness Ra of the plate is 0.3~2.0 µm, and the peak roughness count RPC of the surface of the plate is 30~150;
(3) blanking: performing blanking on the plate or cutting the plate to obtain a blank having a required component shape;
(4) heat treatment: putting the blank into a heating furnace for heating and heat preservation, wherein the temperature of the heating furnace is 880~960 °C, the atmosphere in the heating furnace is air or nitrogen, and the residence time of the blank in the heating furnace is 2.5~10 min, wherein during the heating up process of blank heating, the heating rate does not exceed 10 °C/s in the range of heating up to 400~600 °C;
(5) transferring and hot stamping: quickly transferring the heated blank to a mold for cooling and stamping forming to form a thermoformed component, wherein the blank is transferred to the mold within 20 seconds, the closing speed of the mold during stamping is 30~150 mm/s, and/or the blank is cooled to 50~200 °C at a cooling rate of 30~150 °C/s, wherein after the mold is closed, a pressure holding quenching is continued for 4~20 s, and the pressure holding pressure applied to the blank surface is ≥ 8 MPa, and wherein the material of the mold meets the following requirement: the thermal diffusion coefficient at 700 °C is greater than 3.8 mm²/s.

In the manufacturing method of the present invention, in step (4), too low temperature of the heating furnace or too short residence time of the blank in the heating furnace will lead to insufficient diffusion of iron and aluminum, resulting in too low surface roughness and affecting the roughness of the final thermoformed component. If the temperature of the heating furnace is too high or the residence time of the blank in the heating furnace is too long, it will lead to excessive diffusion of iron and aluminum and complete formation of FeAl alloy, which will also reduce the roughness of the final thermoformed component. At the same time, the holes formed by element migration in the diffusion process will affect the surface conductivity, and cause shrinkage in the electrophoresis process, which will affect the paintability.

Further, in the manufacturing method according to one embodiment of the present invention, in step (1), the mass percentage of chemical elements of the aluminum coating solution is: Si: 8~11%, Fe: 2~4%, Zn: 0~11%, Mg: 0~8%, and a balance of Al and other unavoidable impurities.

Further, in the manufacturing method according to one embodiment of the present invention, the average weight of the aluminum coating is 30~100 g/m² per single surface.

Further, in the manufacturing method of the present invention, in step (4), during the heating up process of blank heating, the heating rate does not exceed 10 °C/s in the range of heating up to 400~600 °C to pre-alloy zinc and aluminum in the coating and avoid damage or crack of the coating.

Further, in the manufacturing method of the present invention, in step (5), the blank is transferred to the mold within 20 seconds.

Further, in the manufacturing method of the present invention, in the hot stamping process of step (5), after the mold is closed, a pressure holding quenching is continued for 4~20 s, and the pressure holding pressure applied to the blank surface is ≥8 MPa. In some embodiments, the pressure holding pressure is 10~20 MPa.

Further, in the manufacturing method of the present invention, in step (5), the material of the mold meets the following requirement: the thermal diffusion coefficient at 700 °C is greater than 3.8 mm²/s.

Further, in the manufacturing method of the present invention, in step (5), during stamping, the closing speed of the mold is 30~150 mm/s, so that the thermoformed component can ensure good forming performance and reduce stamping defects, such as cracking and necking.

Further, in the manufacturing method of the present invention, in step (5), the blank is cooled to 50~200 °C at a cooling rate of 30~150 °C/s to change the internal structure of the thermoformed component into the required structure, and ensure that the thermoformed component still maintains a good size and shape during the cooling process.

The present invention also includes a thermoformed component manufactured by the above method.

Compared with the prior art, the thermoformed component having excellent coating adhesion and its method have the following advantages and beneficial effects:
The thermoformed component having excellent coating adhesion of the present invention has good paintability, good coating adhesion and good corrosion resistance, and is very suitable for automotive parts, such as front and rear doors, left and right anti-collision rods/beams, front and rear bumpers, A-pillar reinforcing plates, B-pillar reinforcing plates, floor middle channels, etc.

In addition, the manufacturing method of the present invention also has the above advantages and beneficial effects.

### DETAILED DESCRIPTION

The thermoformed component having excellent coating adhesion of the present invention and its manufacturing method will be further explained and illustrated with reference to specific examples. Nonetheless, the explanation and illustration are not intended to unduly limit the technical solution of the present invention.

### Examples 1-10 and Comparative Example 1

The thermoformed components having excellent coating adhesion of Examples 1-10 and Comparative Example 1 are manufactured by the following step:
(1) Immersing a substrate in an aluminum coating solution to obtain a plate having an aluminum coating on a surface thereof.
(2) Leveling: using a leveling roller having a roughness Ra of 0.5~3.0 µm to level the plate, and controlling the leveling elongation ≤2.0%, so that the surface thermal radiation coefficient of the plate was 0.1~0.8, the surface roughness Ra of the plate was 0.3~2.0 µm, and the peak roughness count Rpc of the surface of the plate was 30~150.
(3) Blanking: performing blanking on the plate or cutting the plate to obtain a blank having a required component shape;
(4) Heat treatment: putting the blank into a heating furnace for heating and heat preservation, wherein the temperature of the heating furnace was 880~960 °C, the atmosphere in the heating furnace was air or nitrogen, the residence time of the blank in the heating furnace was 2.5~10 min, and during the heating up process of blank heating, the heating rate did not exceed 10 °C/s in the range of heating up to 400~600 °C.
(5) Transferring and hot stamping: quickly (such as within 20 seconds) transferring the heated blank to a mold for cooling and stamping forming to form a thermoformed component. Wherein, in the hot stamping process, after the mold was closed, a pressure holding quenching was continued for 4~20 s, the pressure holding pressure applied to the blank surface was ≥8 MPa, and the material of the mold met the following requirement: the thermal diffusion coefficient at 700 °C was greater than 3.8 mm²/s, and during stamping, the closing speed of the mold was 30~150 mm/s, and the blank was cooled to 50~200 °C at a cooling rate of 30~150 °C/s.

Wherein, the manufacturing methods of every Examples and Comparative Example are as follows:

### Example 1

A 1.2 mm steel plate with aluminum alloy coating was leveled by a leveling roller to obtain a plate before heat treatment and hot stamping having a surface roughness as shown in Table 2, and the plate was laser blanked into a blank with a certain size and shape. The mass percentage of chemical compositions of the aluminum coating solution was Si: 8.5%, Fe: 2.6%, Zn: 15%, Mg: 4%, and a balance of Al and other unavoidable impurities. The blank entered a heating furnace. The temperature of the heating furnace was 950 °C, the residence time was 3.5 minutes, the heating rate was 2 °C/s in the range of 400~600 °C, the transferring time was 4 seconds, the pressure holding time was 5 seconds, the pressure holding pressure was 10 MPa, the mold closing speed was 50 mm/s, the cooling speed was 50 °C/s, the finish temperature of cooling was 200 °C and the thermal diffusion coefficient of the mold at 700 °C was 4 mm²/s.

### Example 2

A 0.9mm steel plate with aluminum alloy coating was leveled by a leveling roller to obtain a plate before heat treatment and hot stamping having a surface roughness as shown in Table 2, and the plate was laser blanked into a blank with a certain size and shape. The mass percentage of chemical compositions of the aluminum coating solution was Si: 5%, Fe: 2.4%, Zn: 8%, Mg: 8%, and a balance of Al and other unavoidable impurities. The blank entered a heating furnace. The temperature of the heating furnace was 940°C, the residence time was 5 minutes, the heating rate was 5°C/s in the range of 400~600 °C, the transferring time was 6 seconds, the pressure holding time was 15 seconds, the pressure holding pressure was 20 MPa, the mold closing speed was 150 mm/s, the cooling speed was 150 °C/s, the finish temperature of cooling was 50°C and the thermal diffusion coefficient of the mold at 700 °C was 5 mm²/s.

### Example 3

A 1.0mm steel plate with aluminum alloy coating was leveled by a leveling roller to obtain a plate before heat treatment and hot stamping having a surface roughness as shown in Table 2, and the plate was laser blanked into a blank with a certain size and shape. The mass percentage of chemical compositions of the aluminum coating solution was Si: 9.0%, Fe: 2.7%, and a balance of Al and other unavoidable impurities. The blank entered a heating furnace. The heating rate of 400~600 °Cwas 5°C/s, the temperature of the heating furnace was 930°C, the residence time was 7 minutes, the heated blank was transferred to a mold within 8 seconds, and the thermal diffusion coefficient of the mold at 700 °C was 7 mm²/s. The mold closing speed was 70 mm/s, the pressure holding time was 6 seconds, the pressure holding pressure was 12 MPa, the cooling speed was 100 °C/s, and the finish temperature of cooling was 100°C The proportion of martensite in the microstructure of the substrate of the thermoformed component is higher than 96%.

### Example 4

A 2.8mm steel plate with aluminum alloy coating was leveled by a leveling roller to obtain a plate before heat treatment and hot stamping having a surface roughness as shown in Table 2, and the plate was laser blanked into a blank with a certain size and shape. The mass percentage of chemical compositions of the aluminum coating solution was Si: 8.8%, Fe: 2.7%, and a balance of Al and other unavoidable impurities. The blank entered a heating furnace. The temperature of the heating furnace was 920 °C, the residence time was 7 minutes, the heating rate of 400-600 °C was 10°C/s, the heated blank was transferred to a mold within 8 seconds, the mold closing speed was 70mm/s, the pressure holding time was 6 seconds, the pressure holding pressure was 15 MPa, the cooling speed was 60°C/s, the finish temperature of cooling was 60°C and the thermal diffusion coefficient of the mold at 700 °C was 6 mm²/s. The proportion of martensite in the microstructure of the substrate of the thermoformed component is higher than 98%.

### Example 5

A 1.1mm steel plate with aluminum alloy coating was leveled by a leveling roller to obtain a plate before heat treatment and hot stamping having a surface roughness as shown in Table 2, and the plate was laser blanked into a blank with a certain size and shape. The mass percentage of chemical compositions of the aluminum coating solution was Si: 10%, Fe: 3.5%, Zn: 2%, Mg: 1%, and a balance of Al and other unavoidable impurities. The blank entered a heating furnace. The temperature of the heating furnace was 935 °C, the residence time was 4.5 minutes, the heating rate was 4°C/s in the range of 400~600 °C, the heated blank was transferred to a mold within 7 seconds, the mold closing speed of upper and lower molds was 80mm/s, the pressure holding time was 5 seconds, the pressure holding pressure was 15 MPa, the thermal diffusion coefficient of the mold at 700 °C was 4 mm²/s and the finish temperature of cooling was 100°C. The proportion of martensite in the microstructure of the substrate of the thermoformed component is higher than 95%.

### Example 6

A 1.5mm steel plate with aluminum alloy coating was leveled by a leveling roller to obtain a plate before heat treatment and hot stamping having a surface roughness as shown in Table 2, and the plate was laser blanked into a blank with a certain size and shape. The mass percentage of chemical compositions of the aluminum coating solution was Si: 10%, Fe: 3.5%, Mg: 0.5%, and a balance of Al and other unavoidable impurities. The blank entered a heating furnace. The temperature of the heating furnace was 935 °C, the residence time was 5 minutes, the heating rate was 6°C/s in the range of 400~600 °C, the heated blank was transferred to a mold within 7 seconds, the mold closing speed of upper and lower molds was 80 mm/s, the pressure holding time was 5 seconds, the pressure holding pressure was 15 MPa, the thermal diffusion coefficient of the mold at 700 °C was 4 mm²/s and the finish temperature of cooling was 120°C. The proportion of martensite in the microstructure of the substrate of the thermoformed component is higher than 95%.

### Example 7

A 1.8mm steel plate with aluminum alloy coating was leveled by a leveling roller to obtain a plate before heat treatment and hot stamping having a surface roughness as shown in Table 2, and the plate was laser blanked into a blank with a certain size and shape. The mass percentage of chemical compositions of the aluminum coating solution was Si: 10%, Fe: 3.5%, and a balance of Al and other unavoidable impurities. The blank entered a heating furnace. The temperature of the heating furnace was 945°C, the residence time was 2.5 minutes, the heating rate was 7°C/s in the range of 400~600 °C, the heated blank was transferred to a mold within 7 seconds, the mold closing speed of upper and lower molds was 80 mm/s, the pressure holding time was 5 seconds, the pressure holding pressure was 15 MPa, the thermal diffusion coefficient of the mold at 700 °C was 6.8 mm²/s and the finish temperature of cooling was 140°C. The proportion of martensite in the microstructure of the substrate of the thermoformed component is higher than 95%.

### Example 8

A 2.0mm steel plate with aluminum alloy coating was leveled by a leveling roller to obtain a plate before heat treatment and hot stamping having a surface roughness as shown in Table 2, and the plate was laser blanked into a blank with a certain size and shape. The mass percentage of chemical compositions of the aluminum coating solution was Si: 10%, Fe: 3.5%, and a balance of Al and other unavoidable impurities. The blank entered a heating furnace. The temperature of the heating furnace was 940°C, the residence time was 3 minutes, the heating rate was 3°C/s in the range of 400~600 °C, the oxygen content of the atmosphere in the furnace was 22%, the heated blank was transferred to a mold within 7 seconds, the mold closing speed of upper and lower molds was 80 mm/s, the pressure holding time was 5 seconds, the pressure holding pressure was 15 MPa, the thermal diffusion coefficient of the mold at 700 °C was 7 mm²/s and the finish temperature of cooling was 110°C. The proportion of martensite in the microstructure of the substrate of the thermoformed component is higher than 95%.

### Example 9

A 2.4mm steel plate with aluminum alloy coating was leveled by a leveling roller to obtain a plate before heat treatment and hot stamping having a surface roughness as shown in Table 2, and the plate was laser blanked into a blank with a certain size and shape. The mass percentage of chemical compositions of the aluminum coating solution was Si: 10%, Fe: 3.5%, and a balance of Al and other unavoidable impurities. The blank entered a heating furnace. The temperature of the heating furnace was 935°C, the residence time was 5 minutes, the heating rate was 8°C/s in the range of 400~600 °C, the oxygen content of the atmosphere in the furnace was 22%, the heated blank was transferred to a mold within 7 seconds, the mold closing speed of upper and lower molds was 80 mm/s, the pressure holding time was 5 seconds, the pressure holding pressure was 15 MPa, the thermal diffusion coefficient of the mold at 700 °C was 4 mm²/s and the finish temperature of cooling was 100°C. The proportion of martensite in the microstructure of the substrate of the thermoformed component is higher than 95%.

### Example 10

A 2.8mm steel plate with aluminum alloy coating was leveled by a leveling roller to obtain a plate before heat treatment and hot stamping having a surface roughness as shown in Table 2, and the plate was laser blanked into a blank with a certain size and shape. The mass percentage of chemical compositions of the aluminum coating solution was Si: 10%, Fe: 3.5%, and a balance of Al and other unavoidable impurities. The blank entered a heating furnace. The temperature of the heating furnace was 950°C, the residence time was 2.5 minutes, the heating rate was 4°C/s in the range of 400~600 °C, the oxygen content of the atmosphere in the furnace was 20%, the heated blank was transferred to a mold within 15 seconds, the mold closing speed of upper and lower molds was 80 mm/s, the pressure holding time was 5 seconds, the pressure holding pressure was 15 MPa, the thermal diffusion coefficient of the mold at 700 °C was 5 mm²/s and the finish temperature of cooling was 80°C. The proportion of martensite in the microstructure of the substrate of the thermoformed component is higher than 95%.

### Comparative Example 1

A 1.5mm steel plate with aluminum alloy coating was leveled by a leveling roller to obtain a plate before heat treatment and hot stamping having a surface roughness as shown in Table 2, and the plate was laser blanked into a blank with a certain size and shape. The mass percentage of chemical compositions of the aluminum coating solution was Si: 10%, Fe: 3.5%, and a balance of Al and other unavoidable impurities. The blank entered a heating furnace. The temperature of the heating furnace was 935°C, the residence time was 5 minutes, the heating rate was 6°C/s in the range of 400~600 °C, the heated blank was transferred to a mold within 7 seconds, the mold closing speed of upper and lower molds was 80 mm/s, the pressure holding time was 5 seconds, the pressure holding pressure was 15 MPa, the thermal diffusion coefficient of the mold at 700 °C was 4 mm²/s and the finish temperature of cooling was 120°C. The proportion of martensite in the microstructure of the substrate of the thermoformed component is higher than 95%.

Table 1 lists the mass percentage ratio of each chemical element of the substrate layers of the thermoformed components having excellent coating adhesion of Examples 1-10 and the substrate layer of Comparative Example 1.

**Table 1. (wt%, and a balance of Fe and other unavoidable impurities)**

| Example | C | Si | Mn | P | S | Al | Ti | B | Cr | Nb | V |
|---|---|---|---|---|---|---|---|---|---|---|---|
| 1 | 0.02 | 0.05 | 0.12 | 0.059 | 0.038 | 0.09 | 0.090 | 0.0005 | 0.15 | - | - |
| 2 | 0.06 | 0.23 | 1.19 | 0.015 | 0.001 | 0.04 | 0.030 | 0.040 | 0.27 | - | - |
| 3 | 0.49 | 0.50 | 2.51 | 0.024 | 0.04 | 0.08 | 0.027 | 0.0052 | 0.51 | 0.002 | 0.002 |
| 4 | 0.39 | 0.36 | 3.00 | 0.044 | 0.03 | 0.07 | 0.05 | 0.0062 | 0.71 | 0.003 | 0.005 |
| 5 | 0.78 | 0.48 | 0.50 | 0.081 | 0.02 | 0.05 | 0.48 | 0.0071 | 0.20 | 0.1 | - |
| 6 | 0.15 | 0.10 | 2.90 | 0.059 | 0.038 | 0.09 | 0.090 | 0.0031 | 0.15 | - | - |
| 7 | 0.25 | 0.23 | 1.19 | 0.015 | 0.001 | 0.04 | 0.030 | 0.0040 | 0.27 | - | - |
| 8 | 0.49 | 0.50 | 2.51 | 0.024 | 0.04 | 0.08 | 0.027 | 0.0052 | 0.51 | 0.005 | 0.008 |
| 9 | 0.39 | 0.36 | 3.00 | 0.044 | 0.03 | 0.07 | 0.05 | 0.0062 | 0.71 | - | - |
| 10 | 0.50 | 0.9 | 0.50 | 0.081 | 0.02 | 0.05 | 0.20 | 0.09 | 0.20 | - | - |
| Comparative Example 1 | 0.25 | 0.23 | 1.19 | 0.015 | 0.001 | 0.04 | 0.030 | 0.0040 | 0.27 | - | - |

To verify the application effect of the present invention and prove the components having excellent coating adhesion of Examples 1-10 and the comparative thermoformed component of Comparative Example 1 were tested in the present invention. Table 2 lists the test results of every Examples and Comparative Example.

**Table 2**

| Example | | 1 | 2 | 3 | 4 | 5 | 6 | 7 | 8 | 9 | 10 | Comparati ve Example 1 |
|---|---|---|---|---|---|---|---|---|---|---|---|---|
| Average weight of aluminum coating, g/m² per surface | | 23 | 30 | 50 | 60 | 100 | 70 | 80 | 85 | 80 | 75 | 75 |
| Thickness, mm | | 1.2 | 0.9 | 1 | 2.8 | 1.1 | 1.5 | 1.8 | 2 | 2.4 | 2.8 | 1.5 |
| Leveling elongation/% | | 0.5 | 0.8 | 1.5 | 0.3 | 0.6 | 0.7 | 1 | 1.2 | 1.8 | 2 | 0.7 |
| Roughness of leveling roller/µm | | 0.5 | 1.2 | 3 | 1 | 1.5 | 1.5 | 1.8 | 1.2 | 1.9 | 2.8 | ***0.3*** |
| Roughness of plate before heat | Ra/µm | 0.3 | 0.8 | 2 | 0.9 | 1.3 | 1 | 1.1 | 0.8 | 0.7 | 1.5 | 0.2 |
| treatment and hot stamping | Rpc | 50 | 90 | 150 | 90 | 50 | 100 | 70 | 130 | 90 | 80 | 25 |
| Roughness of finished product after heat treatment and hot stamping | Ra/µm | 1.8 | 1.8 | 1.9 | 2 | 2.3 | 2 | 1.9 | 1.9 | 1.8 | 2.4 | 1.3 |
| | Rt/µm | 12 | 13 | 18 | 19 | 20 | 21 | 18 | 19 | 19 | 22 | 9 |
| | Rpc | 90 | 100 | 120 | 120 | 160 | 170 | 150 | 160 | 140 | 170 | ***40*** |
| Thickness of 50% Al layer in alloy layer/µm | | 15 | 18 | 20 | 25 | 35 | 26 | 20 | 28 | 26 | 20 | 20 |
| Thickness of diffusion layer/µm | | 5 | 6 | 7 | 8 | 16 | 10 | 8 | 8 | 8 | 8 | 8 |
| Thickness of total aluminum coating/µm | | 22 | 25 | 30 | 33 | 60 | 40 | 35 | 40 | 38 | 30 | 30 |
| Tensile strength of product after stamping/MPa | | 500 | 700 | 1820 | 2000 | 1900 | 1000 | 1550 | 1590 | 1600 | 1580 | 1500 |
| Yield strength of product after stamping/MPa | | 400 | 500 | 1250 | 1350 | 1200 | 1050 | 1000 | 980 | 1100 | 1100 | 1100 |
| Elongation/% | | 19 | 15 | 5 | 4 | 4.5 | 6 | 7 | 6 | 6 | 6 | 6 |
| Paintability | | The surface of the coating is uniform after pretreatment | | | | | | | | | | Nonunifor m |
| Coating adhesion after coating | | Grad e 1 | Grad e 1 | Grade 2 | Grade 2 | Grade 1 | Grade 1 | Grade 2 | Grade 1 | Grade 2 | Grade 1 | Grade 5 |
| Corrosion resistance, mm | | 1 | 1.5 | 3 | 3.5 | 2 | 2.3 | 3.5 | 3 | 3.8 | 3 | 5 |

| | | | | | | | | | | | | |
|---|---|---|---|---|---|---|---|---|---|---|---|---|
| *Test method for coating adhesion: Referring to GB/T 9286-1998 cross cut test method, cutting grids on the surface with a knife, sticking an adhesive tape to the center of the formed grids, then pulling it off smoothly, observing the phenomenon of coating falling off, and judging the grade by calculating the state of grids according to the standard. The paintability was evaluated with reference to GMW16170 standard. The corrosion resistance was tested with reference to GMW14872. | | | | | | | | | | | | |

As can be seen from Table 2, the yield strength of each example of the present invention is 400~1350 MPa, the tensile strength is 500~2000 MPa, and the elongation is 4~19%.

In addition, it can be seen from Table 2 that the surface roughness Ra of the finished product of the comparative thermoformed component of Comparative Example 1 after hot stamping is lower than 1.8 µm, Rt is less than 12 µm, Rpc is lower than 90, and the paintability of the thermoformed component of Comparative Example 1 is poor, the coating adhesion does not meet the requirements, and its performance is far inferior to that of the thermoformed components of every Examples of the present invention. In addition, it can be seen from table 2 that the higher the surface roughness of the material before heat treatment and hot stamping used by the thermoformed component, the higher the product roughness after heat treatment and hot stamping, and the better the coating adhesion.

To sum up, the thermoformed component having excellent coating adhesion of the present invention has good paintability, good coating adhesion and good corrosion resistance, and is very suitable for automotive parts, such as front and rear doors, left and right anti-collision rods/beams, front and rear bumpers, A-pillar reinforcing plates, B-pillar reinforcing plates, floor middle channels, etc.

In addition, the manufacturing method of the present invention also has the above advantages and beneficial effects.

It should be noted that the examples listed above are only specific examples of the present invention. Obviously, the present invention is not limited to the above examples.

## Claims

1. A thermoformed component having excellent coating adhesion, comprising a substrate layer and an aluminum coating coated on at least one surface of the substrate layer, wherein the average roughness Ra of a surface of the thermoformed component is 1.0~3.0 µm, the peak-to-valley height Rt is 8~30 µm, and the roughness peak count Rpc is ≥50, wherein the mass percentage of chemical elements of the aluminum coating is: Si: 4~14%, Fe: 0~4%, Mg: 0~10%, Zn: 0~20%, and a balance of Al and other unavoidable impurities, wherein the aluminum coating comprises a diffusion layer adjacent to the substrate layer and an alloy layer on the surface of the aluminum coating, wherein the ratio of the thickness of the diffusion layer to the total thickness of the aluminum coating is 0.08-0.5, and
wherein the mass percentage of chemical elements of the substrate layer is:
C: 0.01 -0.8%, Si: 0.05~1.0%, Mn: 0.1~5%, P≤0.3%, S≤0.1%, Al<0.3%, Ti≤0.5%, B: 0.0005~0.1%, Cr: 0.01 ~3%, Nb≤0.5%, V≤0.5%, and a balance of Fe and other unavoidable impurities.

2. The thermoformed component having excellent coating adhesion according to claim 1 or 2, wherein the thickness of the diffusion layer is ≤16 µm, and the total thickness of the aluminum coating is ≤60 µm.

3. The thermoformed component having excellent coating adhesion according to claim 1, wherein the mass percentage of chemical elements of the aluminum coating is: Si: 4~14%, Fe: 2~4%, Mg: 0~10%, Zn: 0~20%, and a balance of Al and other unavoidable impurities.

4. The thermoformed component having excellent coating adhesion according to claim 1, wherein the mass percentage of chemical elements of the substrate layer further meets at least one of the following:
C: 0.05-0.6%,
Si: 0.07~0.8%,
Mn: 0.3~4%,
P≤0.2%,
S≤0.08%,
Al≤0.2%,
Ti≤0.4%,
B: 0.0005~0.08%,
Cr: 0.01 ~2%,
Nb≤0.3%,
V≤0.3%;
preferably, the mass percentage of chemical elements of the substrate layer further meets at least one of the following:
C: 0.15~0.5%,
Si: 0.1~0.5%,
Mn: 0.5~3%,
P≤0.1%,
S≤0.05%,
Al≤0.1%,
Ti≤0.2%,
Cr: 0.01~1%.

5. The thermoformed component having excellent coating adhesion according to claim 1, wherein the yield strength of the thermoformed component having excellent coating adhesion is 400~1400 MPa, the tensile strength is 500~2100 MPa, and the elongation is ≥4%.

6. The thermoformed component having excellent coating adhesion according to claim 1, wherein the surface of the thermoformed component having excellent coating adhesion comprises Fe₂Al₅ and FeAl alloy; or the surface of the thermoformed component having excellent coating adhesion mainly consists of Fe₂Al₅ and FeAl alloy, and further comprises silicon oxide, aluminum oxide and iron oxide.

7. The thermoformed component having excellent coating adhesion according to claim 4, wherein the volume percentage of martensite in the microstructure of the substrate layer of the thermoformed component having excellent coating adhesion is ≥95%.

8. A manufacturing method for the thermoformed component having excellent coating adhesion of any one of claims 1-7, comprising the following steps:
(1) immersing a substrate in an aluminum coating solution to obtain a plate having an aluminum coating on a surface thereof, wherein the average weight of the aluminum coating is 20~120 g/m² per single surface, wherein the mass percentage of chemical elements of the substrate is: C: 0.01-0.8%, Si: 0.05~1.0%, Mn: 0.1 ~5%, P≤0.3%, S≤0.1%, Al<0.3%, Ti≤0.5%, B: 0.0005~0.1%, Cr: 0.01 ~3%, Nb≤0.5%, V≤0.5%, and a balance of Fe and other unavoidable impurities, and wherein the mass percentage of chemical elements of the aluminum coating solution is: Si: 5~11%, Fe: 2~4%, Zn: 0~15%, Mg: 0~8%, and a balance of Al and other unavoidable impurities;
(2) leveling: using a leveling roller having a roughness Ra of 0.5~3.0 µm to level the plate, and controlling the leveling elongation ≤2.0%, wherein the surface thermal radiation coefficient of the plate is 0.1~0.8, the surface roughness Ra of the plate is 0.3~2.0 µm, and the peak roughness count RPC of the surface of the plate is 30~150;
(3) blanking: performing blanking on the plate or cutting the plate to obtain a blank having a required component shape;
(4) heat treatment: putting the blank into a heating furnace for heating and heat preservation, wherein the temperature of the heating furnace is 880~960 °C, the atmosphere in the heating furnace is air or nitrogen, and the residence time of the blank in the heating furnace is 2.5~10 min, wherein during the heating up process of blank heating, the heating rate does not exceed 10 °C/s in the range of heating up to 400~600 °C;
(5) transferring and hot stamping: quickly transferring the heated blank to a mold for cooling and stamping forming to form the thermoformed component, wherein the blank is transferred to the mold within 20 seconds, the closing speed of the mold during stamping is 30~150 mm/s, and/or the blank is cooled to 50~200 °C at a cooling rate of 30~150 °C/s, wherein after the mold is closed, a pressure holding quenching is continued for 4~20 s, and the pressure holding pressure applied to the blank surface is ≥ 8 MPa, and wherein the material of the mold meets the following requirement: the thermal diffusion coefficient at 700 °C is greater than 3.8 mm²/s.

9. The manufacturing method according to claim 8, wherein the average weight of the aluminum coating is 30~100 g/m² per single surface.

## Patentansprüche

1. Eine thermogeformte Komponente mit ausgezeichneter Beschichtungshaftung, umfassend eine Substratschicht und eine Aluminiumbeschichtung, die auf mindestens eine Oberfläche der Substratschicht aufgebracht ist, wobei die durchschnittliche Rauheit Ra einer Oberfläche der thermogeformten Komponente 1,0 bis 3,0 µm beträgt, die Spitze-Tal-Höhe Rt 8 bis 30 µm beträgt und der Spitzenrauheitswert Rpc ≥ 50 ist, wobei der Massenanteil der chemischen Elemente der Aluminiumbeschichtung wie folgt ist: Si: 4 bis 14 %, Fe: 0 bis 4 %, Mg: 0 bis 10 %, Zn: 0 bis 20 % und der Rest Al und andere unvermeidbare Verunreinigungen ist, wobei die Aluminiumbeschichtung eine an die Substratschicht angrenzende Diffusionsschicht und eine Legierungsschicht auf der Oberfläche der Aluminiumbeschichtung umfasst, wobei das Verhältnis der Dicke der Diffusionsschicht zur Gesamtdicke der Aluminiumbeschichtung 0,08 bis 0,5 beträgt, und
wobei der Massenanteil der chemischen Elemente der Substratschicht wie folgt ist:
C: 0,01 bis 0,8 %, Si: 0,05 bis 1,0 %, Mn: 0,1 bis 5 %, P ≤ 0,3 %, S ≤ 0,1 %, Al ≤ 0,3 %, Ti ≤ 0,5 %, B:
0,0005 bis 0,1 %, Cr: 0,01 bis 3 %, Nb ≤ 0,5 %, V ≤ 0,5 % und der Rest Fe und andere unvermeidbare Verunreinigungen ist.

2. Die thermogeformte Komponente mit ausgezeichneter Beschichtungshaftung gemäß Anspruch 1 oder 2, wobei die Dicke der Diffusionsschicht ≤ 16 µm beträgt und die Gesamtdicke der Aluminiumbeschichtung ≤ 60 µm beträgt.

3. Die thermogeformte Komponente mit ausgezeichneter Beschichtungshaftung gemäß Anspruch 1, wobei der Massenanteil der chemischen Elemente der Aluminiumbeschichtung wie folgt ist: Si: 4 bis 14 %, Fe: 2 bis 4 %, Mg: 0 bis 10 %, Zn: 0 bis 20 % und der Rest Al und andere unvermeidbare Verunreinigungen ist.

4. Die thermogeformte Komponente mit ausgezeichneter Beschichtungshaftung gemäß Anspruch 1, wobei der Massenanteil der chemischen Elemente der Substratschicht zusätzlich mindestens eine der folgenden Bedingungen erfüllt:
C: 0,05 bis 0,6 %,
Si: 0,07 bis 0,8 %,
Mn: 0,3 bis 4 %,
P ≤ 0,2 %,
S ≤ 0,08 %,
Al ≤ 0,2 %,
Ti ≤ 0,4 %,
B: 0,0005 bis 0,08 %,
Cr: 0,01 bis 2 %,
Nb ≤ 0,3 %,
V ≤ 0,3 %;
vorzugsweise erfüllt der Massenanteil der chemischen Elemente der Substratschicht mindestens eine der folgenden Bedingungen:
C: 0,15 bis 0,5 %,
Si: 0,1 bis 0,5 %,
Mn: 0,5 bis 3 %,
P ≤ 0,1 %,
S ≤ 0,05 %,
Al ≤ 0,1 %,
Ti ≤ 0,2 %,
Cr: 0,01 bis 1 %.

5. Die thermogeformte Komponente mit ausgezeichneter Beschichtungshaftung gemäß Anspruch 1, wobei die Streckgrenze der thermogeformten Komponente mit ausgezeichneter Beschichtungshaftung 400 bis 1400 MPa beträgt, die Zugfestigkeit 500 bis 2100 MPa beträgt und die Dehnung ≥ 4 % beträgt.

6. Die thermogeformte Komponente mit ausgezeichneter Beschichtungshaftung gemäß Anspruch 1, wobei die Oberfläche der thermogeformten Komponente mit ausgezeichneter Beschichtungshaftung Fe₂Al₅ und eine FeAl-Legierung umfasst; oder die Oberfläche der thermogeformten Komponente mit ausgezeichneter Beschichtungshaftung hauptsächlich aus Fe₂Al₅ und einer FeAl-Legierung besteht und zusätzlich Siliziumoxid, Aluminiumoxid und Eisenoxid umfasst.

7. Die thermogeformte Komponente mit ausgezeichneter Beschichtungshaftung gemäß Anspruch 4, wobei der Volumenanteil an Martensit in der Mikrostruktur der Substratschicht der thermogeformten Komponente mit ausgezeichneter Beschichtungshaftung ≥ 95 % beträgt.

8. Verfahren zur Herstellung einer thermogeformten Komponente mit ausgezeichneter Beschichtungshaftung gemäß einem der Ansprüche 1 bis 7, umfassend die folgenden Schritte:
(1) Eintauchen eines Substrats in eine Aluminiumbeschichtungslösung, um eine Platte mit einer Aluminiumbeschichtung auf einer Oberfläche davon zu erhalten, wobei das durchschnittliche Gewicht der Aluminiumbeschichtung 20 bis 120 g/m² pro Oberfläche beträgt, wobei der Massenanteil der chemischen Elemente des Substrats wie folgt ist: C: 0,01 bis 0,8 %, Si: 0,05 bis 1,0 %, Mn: 0,1 bis 5 %, P ≤ 0,3 %, S ≤ 0,1 %, Al ≤ 0,3 %, Ti ≤ 0,5 %, B: 0,0005 bis 0,1 %, Cr: 0,01 bis 3 %, Nb ≤ 0,5 %, V ≤ 0,5 % und der Rest Fe und anderen unvermeidbaren Verunreinigungen ist, und wobei der Massenanteil der chemischen Elemente der Aluminiumbeschichtungslösung wie folgt ist: Si: 5 bis 11 %, Fe: 2 bis 4 %, Zn: 0 bis 15 %, Mg: 0 bis 8 % und der Rest Al und andere unvermeidbare Verunreinigungen ist;
(2) Nivellierung: Verwenden einer Nivellierwalze mit einer Rauheit Ra von 0,5 bis 3,0 µm zum Nivellieren der Platte und Steuern der Nivellierungsdehnung auf ≤ 2,0 %, wobei der Oberflächenwärmestrahlungskoeffizient der Platte 0,1 bis 0,8 beträgt, die Oberflächenrauheit Ra der Platte 0,3 bis 2,0 µm beträgt und der Spitzenrauheitswert RPC der Oberfläche der Platte 30 bis 150 beträgt;
(3) Stanzen: Stanzen der Platte oder Schneiden der Platte, um einen Rohling mit der erforderlichen Form zu erhalten;
(4) Wärmebehandlung: Einlegen des Rohlings in einen Heizofen zum Erhitzen und Warmhalten, wobei die Temperatur des Heizofens 880 bis 960 °C beträgt, die Atmosphäre im Heizofen ist Luft oder Stickstoff und die Verweildauer des Rohlings im Heizofen beträgt 2,5 bis 10 Minuten, wobei während des Aufheizvorgangs des Rohlings die Aufheizgeschwindigkeit im Bereich von 400 bis 600 °C 10 °C/s nicht überschreitet;
(5) Übertragen und Heißprägen: schnelles Übertragen des erhitzten Rohlings in eine Form zum Abkühlen und Prägen, um die thermogeformte Komponente zu formen, wobei der Rohling innerhalb von 20 Sekunden in die Form übertragen wird, die Schließgeschwindigkeit der Form während des Prägen 30 bis 150 mm/s beträgt und/oder der Rohling auf 50 bis 200 °C abgekühlt wird mit einer Abkühlgeschwindigkeit von 30 bis 150 °C/s, wobei nach dem Schließen der Form eine Druckhalteabschreckung für 4 bis 20 s fortgesetzt wird und der auf die Rohlingsoberfläche ausgeübte Druckhaltewert ≥ 8 MPa beträgt, und wobei das Material der Form die folgende Anforderung erfüllt: Der Wärmediffusionskoeffizient bei 700 °C ist größer als 3,8 mm²/s.

9. Das Verfahren zur Herstellung gemäß Anspruch 8, wobei das durchschnittliche Gewicht der Aluminiumbeschichtung 30 bis 100 g/m² pro Oberfläche beträgt.

## Revendications

1. Composant thermoformé présentant une excellente adhérence du revêtement, comprenant une couche de substrat et un revêtement en aluminium appliqué sur au moins une surface de la couche de substrat, dans laquelle la rugosité moyenne Ra d'une surface du composant thermoformé est de 1,0 à 3,0 µm, la hauteur de crête à vallée Rt est de 8 à 30 µm, et le nombre de pics de rugosité Rpc est ≥ 50, dans lequel le pourcentage massique des éléments chimiques du revêtement en aluminium est : Si : 4 à 14 %, Fe : 0 à 4 %, Mg : 0 à 10 %, Zn : 0 à 20 %, et le reste étant constitué d'Al et d'autres impuretés inévitables, dans lequel le revêtement d'aluminium comprend une couche de diffusion adjacente à la couche de substrat et une couche d'alliage sur la surface du revêtement d'aluminium, dans lequel le rapport entre l'épaisseur de la couche de diffusion et l'épaisseur totale du revêtement d'aluminium est de 0,08 à 0,5, et
dans lequel le pourcentage massique des éléments chimiques de la couche de substrat est le suivant :
C : 0,01 à 0,8 %, Si : 0,05 à 1,0 %, Mn : 0,1 à 5 %, P ≤ 0,3 %, S ≤ 0,1 %, Al ≤ 0,3 %, Ti ≤ 0,5 %, B : 0,0005 à 0,1 %, Cr : 0,01 à 3 %, Nb ≤ 0,5 %, V ≤ 0,5 %, et le reste étant constitué de Fe et d'autres impuretés inévitables.

2. Le composant thermoformé présentant une excellente adhérence du revêtement selon la revendication 1 ou 2, dans lequel l'épaisseur de la couche de diffusion est ≤ 16 µm et l'épaisseur totale du revêtement en aluminium est ≤ 60 µm.

3. Le composant thermoformé présentant une excellente adhérence du revêtement selon la revendication 1, dans lequel le pourcentage massique des éléments chimiques du revêtement d'aluminium est le suivant : Si : 4 à 14 %, Fe : 2 à 4 %, Mg : 0 à 10 %, Zn : 0 à 20 %, et le reste étant constitué d'Al et d'autres impuretés inévitables.

4. Le composant thermoformé présentant une excellente adhérence du revêtement selon la revendication 1, dans lequel le pourcentage massique des éléments chimiques de la couche de substrat satisfait en outre à au moins l'une des conditions suivantes :
C : 0,05 à 0,6 %,
Si : 0,07 à 0,8 %,
Mn : 0,3 à 4 %,
P ≤ 0,2 %,
S ≤ 0,08 %,
Al ≤ 0,2 %,
Ti ≤ 0,4 %,
B : 0,0005 à 0,08 %,
Cr : 0,01 à 2 %,
Nb ≤ 0,3 %,
V ≤ 0,3 % ;
de préférence, le pourcentage massique des éléments chimiques de la couche de substrat satisfait en outre à au moins l'une des conditions suivantes :
C : 0,15 à 0,5 %,
Si : 0,1 à 0,5 %,
Mn : 0,5 à 3 %,
P ≤ 0,1 %,
S ≤ 0,05 %,
Al ≤ 0,1 %,
Ti ≤ 0,2 %,
Cr : 0,01 à 1 %.

5. Le composant thermoformé présentant une excellente adhérence du revêtement selon la revendication 1, dans lequel la limite d'élasticité du composant thermoformé présentant une excellente adhérence du revêtement est de 400 à 1400 MPa, la résistance à la traction est de 500 à 2100 MPa et l'allongement est ≥ 4 %.

6. Le composant thermoformé présentant une excellente adhérence du revêtement selon la revendication 1, dans lequel la surface du composant thermoformé présentant une excellente adhérence du revêtement comprend du Fe₂Al₅ et un alliage de FeAl ; ou la surface du composant thermoformé présentant une excellente adhérence du revêtement est principalement constituée de Fe₂Al₅ et d'un alliage de FeAl, et comprend en outre de l'oxyde de silicium, de l'oxyde d'aluminium et de l'oxyde de fer.

7. Le composant thermoformé présentant une excellente adhérence du revêtement selon la revendication 4, dans lequel le pourcentage en volume de martensite dans la microstructure de la couche de substrat du composant thermoformé présentant une excellente adhérence du revêtement est ≥ 95 %.

8. Procédé de fabrication d'un composant thermoformé présentant une excellente adhérence du revêtement selon l'une des revendications 1 à 7, comprenant les étapes suivantes :
(1) immerger un substrat dans une solution de revêtement d'aluminium afin d'obtenir une plaque présentant un revêtement d'aluminium sur une surface de celle-ci, dans lequel le poids moyen du revêtement d'aluminium est de 20 à 120 g/m² par surface unique, dans lequel le pourcentage massique des éléments chimiques du substrat est le suivant : C : 0,01 à 0,8 %, Si : 0,05 à 1,0 %, Mn : 0,1 à 5 %, P ≤ 0,3 %, S ≤ 0,1 %, Al ≤ 0,3 %, Ti ≤ 0,5 %, B : 0,0005 à 0,1 %, Cr : 0,01 à 3 %, Nb ≤ 0,5 %, V ≤ 0,5 %, et le reste étant du Fe et d'autres impuretés inévitables, et dans lequel le pourcentage massique des éléments chimiques de la solution de revêtement d'aluminium est : Si : 5 à 11 %, Fe : 2 à 4 %, Zn : 0 à 15 %, Mg : 0 à 8 %, et le reste étant constitué d'AI et d'autres impuretés inévitables ;
(2) nivellement : à l'aide d'un rouleau de nivellement ayant une rugosité Ra de 0,5 à 3,0 µm pour niveler la plaque, et en contrôlant l'allongement de nivellement ≤ 2,0 %, dans lequel le coefficient de rayonnement thermique de surface de la plaque est de 0,1 à 0,8, la rugosité de surface Ra de la plaque est comprise entre 0,3 et 2,0 µm, et le nombre de pics de rugosité RPC de la surface de la plaque est de 30 à 150 ;
(3) découpage : réaliser le découpage de la plaque ou couper la plaque pour obtenir une ébauche ayant la forme requise ;
(4) traitement thermique : placer l'ébauche dans un four de chauffage pour le chauffage et la conservation de la chaleur, la température du four de chauffage étant de 880 à 960 °C, l'atmosphère dans le four de chauffage est de l'air ou de l'azote, et le temps de séjour de l'ébauche dans le four de chauffage est de 2,5 à 10 minutes, dans lequel, pendant le processus de chauffage de l'ébauche, la vitesse de chauffage ne dépasse pas 10 °C/s dans la plage de chauffage de 400 à 600 °C ;
(5) transfert et estampage à chaud : transfert rapide de l'ébauche chauffée vers un moule pour refroidissement et estampage afin de former le composant thermoformé, dans lequel l'ébauche est transférée vers le moule en moins de 20 secondes, la vitesse de fermeture du moule pendant l'estampage est de 30 à 150 mm/s, et/ou l'ébauche est refroidie à une température de 50 à 200 °C à une vitesse de refroidissement de 30 à 150 °C/s, dans lequel, après la fermeture du moule, un refroidissement rapide sous pression est maintenu pendant 4 à 20 s, et la pression de maintien appliquée à la surface de l'ébauche est ≥ 8 MPa, et dans lequel le matériau du moule répond à l'exigence suivante : le coefficient de diffusion thermique à 700 °C est supérieur à 3,8 mm²/s.

9. Le procédé de fabrication selon la revendication 8, dans lequel le poids moyen du revêtement en aluminium est de 30 à 100 g/m² par surface unique.
